

## UNITED STATES PATENT OFFICE

2,104,491

## ADHESIVE

Robert S. McKinney, Chevy Chase, Md., dedicated to the free use of the People of the United States of America

No Drawing. Application July 12, 1937,  
Serial No. 153,197

1 Claim. (Cl. 167—42)

(Granted under the act of March 3, 1883, as amended April 30, 1928; 370 O. G. 757)

This application is made under the act of March 3, 1883, as amended by the act of April 30, 1928, and the invention herein described and claimed, if patented, may be manufactured and used by or for the Government of the United States for governmental purposes without the payment to me of any royalty thereon.

I hereby dedicate the invention herein described to the free use of the People of the United States of America to take effect on the granting of a patent to me.

My invention relates to a new adhesive material which has certain water-resistant properties.

In my studies of tung oil fatty acids, and particularly alpha-eleostearic acid, the principal acid derived from tung oil, I have found that these acids, and particularly alpha-eleostearic acid, when spread out in a thin layer, underwent a change to form an extremely sticky compound. This change, although accelerated by increased temperature and sunlight, takes place more slowly even in the icebox and/or in the dark. After this change has taken place, this sticky compound exhibits certain water-resistant properties.

In the practice of this invention, commercial raw tung oil is saponified with the requisite amount of 15° Baumé sodium hydroxide and the resulting soap is broken up with a slight excess of dilute muriatic acid. The resultant mixture is heated until the fatty acids separate in a clear upper layer. The lower mineral acid layer is

drawn off and the remaining fatty acids washed with warm water until free of mineral acid. The separated fatty acids can be used as such or they may be used in solution in organic solvent. They can also be used as their soluble soaps, the fatty acids being liberated by the application of a second solution of a dilute acid of sufficient strength to liberate the fatty acids.

These tung oil fatty acids or their compounds or solutions are useful as an addition to insecticide or fungicide sprays and powders in that they will adhere to vegetative growth and will not be washed off easily by rain. This material could be mixed with the insecticide or fungicide spray or dust, or its solution could be applied to the vegetation, to be followed later by the desired dust or spray. The soap solution of the tung oil fatty acids could be applied in water solution, to be followed later by a dilute acid solution of sufficient strength to liberate the tung oil fatty acids, or to be followed by the soluble salts of the heavier metals, thereby liberating the insoluble salts of the heavier metals which likewise have adhesive properties.

Having thus described my invention, what I claim for Letters Patent is—

I claim:

An adhesive adapted for use in combination with insecticides and fungicides containing as its essential active ingredient alpha-eleostearic acid.

ROBERT S. MCKINNEY.